

# United States Patent

MacDonald et al.

[15] 3,671,423

[45] June 20, 1972

[54] **STABILIZING HYDROCRACKED LUBRICATING OILS**

[72] Inventors: **John M. MacDonald; Ian D. Campbell**,  
both of Sarnia, Ontario, Canada

[73] Assignee: **Esso Research and Engineering Company**

[22] Filed: **March 16, 1970**

[21] Appl. No.: **20,134**

[52] U.S. Cl.....**208/97, 252/412, 208/99**  
[51] Int. Cl.....**C10g 37/00**  
[58] Field of Search.....**208/99, 97, 96, 18, 28**

[56]

**References Cited**

**UNITED STATES PATENTS**

|           |         |                            |        |
|-----------|---------|----------------------------|--------|
| 3,243,366 | 3/1966  | Kimberlin, Jr. et al. .... | 208/28 |
| 3,438,887 | 4/1969  | Morris et al. ....         | 208/97 |
| 3,005,768 | 10/1961 | Burke .....                | 208/28 |

*Primary Examiner—Delbert E. Gantz  
Assistant Examiner—G. J. Crasanakis  
Attorney—Pearlman and Stahl and C. D. Stores*

[57]

**ABSTRACT**

The instability of lubricating oils to light and air formed by hydrocracking high boiling fractions is removed by percolating the oil through silica-alumina gels containing a Y-type molecular sieve.

**16 Claims, No Drawings**

## STABILIZING HYDROCRACKED LUBRICATING OILS

## BACKGROUND OF THE INVENTION

This invention relates to the preparation of lubricating oils stable to light and air.

For many years, lubricating oils have been obtained from crude oils of various character mainly by separation processes. In order to obtain lubricants of relatively high viscosity index (V.I.), it has been the practice to subject the oils fractionated from the crude to solvent extraction to remove components serving to lower the V.I. The solvent extracted lubricants are naturally resistant to degradation in light and air; however, they are generally fortified with one or more additives in order to improve their resistance to oxidation during use and the like.

Recently it has been discovered that lubricating oils may be produced by hydrocracking. In this conversion process, a heavy petroleum oil is contacted with hydrogen at elevated temperature and pressure in the presence of a hydrocracking catalyst. The hydrocracked product is separated into materials boiling in different temperature ranges, including the lubricating oil boiling range, i.e., oils boiling above 650° F. The lubricating oil fractions differ from those obtained by fractional distillation of crude oils and the like, since they have relatively high V.I. values and thus do not require solvent extraction to enhance their V.I. values.

Unfortunately, however, such lubricating oil fractions suffer from the shortcoming that they are unstable when exposed to light (particularly, actinic rays) and air. When so exposed, sediment, sludge, and lacquer formation occur. There is also a marked darkening in the color of the oil. All of this results in the lessening of the commercial value of such lubricants.

## SUMMARY OF THE INVENTION

It has now been discovered that when lubricating oils produced by hydrocracking are percolated through silica-alumina gels containing a Y-type molecular sieve, there is obtained an unexpectedly high yield of significantly more stable premium grade oil. It appears that the oxide gel containing the zeolite selectively removes the instability-causing compounds from the hydrocracked product without affecting the desirable lubricating oil components.

Broadly stated, this invention comprises subjecting a lubricating oil fraction which is unstable to light and air to a treatment which comprises percolating it through a column of a silica-alumina gel containing a Y-type zeolitic sieve. Such zeolitic materials are commonly used as fluid catalytic cracking catalysts. More specifically the invention covers contacting a high boiling hydrocarbon material with hydrogen in the presence of a hydrocracking catalyst at a temperature in the range of 700° to 900° F. and at an elevated pressure in order to convert at least 10 weight percent of the high-boiling hydrocarbons to products boiling below 650° F., recovering a lubricating oil fraction and percolating said lubricating oil fraction through a column of a zeolitic fluid catalytic cracking catalyst.

## DESCRIPTION OF SPECIFIC EMBODIMENTS

## Hydrocarbon Feed

The hydrocarbon feed material or fractions which can be hydrocracked as described herein, can be substantially any hydrocarbon feed material susceptible to treatment with hydrogen. Generally, however, it is preferred to use high boiling range materials derived from petroleum crude oils, boiling above about 650° F., e.g., heavy gas oils, residual stocks, cycled stocks, topped crudes, reduced crudes, deasphalted residua, and relatively high boiling hydrocarbon fractions derived from coal, tars, pitches, asphalts and shale oils. These materials can be obtained by fractionation, as by vacuum distillation, or crude oils identified by their source, viz: Pennsylvania, Mid-Continent, Gulf Coast, West Texas, Western Canada, Venezuela, Amal, Kuwait, Barco, Safaniya, Alaskan, etc.

## Hydrocracking Catalyst

The catalyst employed in the hydrocracking reaction may include any type of hydrogenation catalyst having cracking activity. Accordingly the catalysts may include the oxides and sulfides of the metals of Group VIB of the Periodic Table or mixtures thereof, such as chromium sulfide, molybdenum sulfide and tungsten sulfide; oxides and sulfides of Group VIII of the Periodic Table or mixtures thereof, such as sulfides of iron, cobalt, nickel, palladium, platinum, rhodium, osmium, and iridium; mixtures of the above oxides and sulfides of the metals of Group VB, VIB, and VIII such as mixtures of nickel sulfide and tungsten sulfide, cobalt and molybdenum oxide or sulfide. The hydrogenating component is deposited on a cracking component, preferably containing a siliceous cracking component such as silica-alumina, silica-magnesia, silica-zirconia, and silica-alumina-zirconia. A zeolitic cracking base may be used instead. For example, a particularly effective hydrocracking catalyst comprises a palladium hydrogenation component composited with a hydrogen faujasite cracking base. Another suitable catalyst comprises a mixture of Group VIB and VIII non-noble metals, such as nickel and tungsten supported on a hydrogen form of crystalline aluminosilicate zeolite with or without clay.

## Hydrogen

Pure hydrogen can be used. However hydrogen of lower purity obtained by recycle from other hydrogenating process or from other refining operations, e.g., reforming, may be used. The hydrogen may be circulated at a rate in the range of from about 1,000 to 20,000 standard cubic feet per barrel of hydrocarbon charge and preferably 5,000 to 20,000 standard cubic feet per barrel of charge. A hydrogen consumption of 1,000 standard cubic feet per barrel of feed is preferred but much more or less may be used.

## Hydrocracking Conditions

The hydrocarbon feed is contacted with hydrogen and a catalyst of the character described above, at a temperature ranging from 500° to 1,000° F., preferably 700° to 900° F. and more preferably below 850° F. The pressure normally ranges above 1,500 psig and the hydrocarbon reactant space velocity through the catalyst is below 1.0 liquid hourly space velocity (V/V/Hr.). It is preferred to maintain the pressure above 2,000 psig, the temperature below 850° F. and the space velocity between 0.1 and 0.75.

The reaction may be carried out in any of the suitable equipment well known in the art for such catalytic operations and may be either batch or continuous. Conversions may range from 10 to 75 percent by volume of products boiling below 650° F.

## Hydrogenated Product Fractionation

Following the hydrocracking reaction, products are withdrawn and passed through a heat exchanger or other suitable cooling device, where they are cooled to a temperature where hydrogen gas can be separated. The cooled effluent is then passed into a high pressure gas separator from which the gases are removed and the liquid product is passed to a fractionator from which several fractions are obtained, including lubricating oil fractions boiling above 650° F.

The lubricating oil fractions may be dewaxed, if desired, by any conventional method to provide an oil having a pour below about 30° F.

## The Percolating Step

The hydrocracked lube oil is then percolated through a column of a zeolite containing fluid catalytic cracking catalyst. The percolating step is best carried out at room temperature but any temperature up to 150° F. can be used. Higher temperatures do not give the desired results.

The zeolitic material through which the oil is percolated may contain any Y-zeolites, i.e., a zeolite having a silica/Al<sub>2</sub>O<sub>3</sub> ratio greater than 3/1. Suitable zeolitic material includes a physical mixture of a conventional amorphous cracking catalyst containing a major amount of silica and a minor amount of alumina and a crystalline aluminosilicate zeolite in a siliceous matrix, e.g., faujasite having uniform pore openings of about 6 to 15 Angstrom units. A particularly suitable catalyst consists of 95 percent of a mixture of 13% Al<sub>2</sub>O<sub>3</sub> and

87%  $\text{SiO}_2$  with 5 percent of 13 Y-zeolite or faujasite. The zeolite-y is first ammonia exchanged, then spray dried and then rare-earth exchanged. These catalysts are described in application Ser. No. 744,287 filed June 12, 1968 for Robbins et al. which is incorporated herein by reference.

#### Illustrative Examples

The following examples illustrate and, in no sense, limit the invention.

#### EXAMPLE 1

A West Texas feedstock consisting of a blend of deasphalted residuum and high vacuum gas oil was hydrocracked at 780° F., 0.5 liquid hourly space velocity and 2,500 psig over a sulfided commercial hydrocracking catalyst. A 10-grade lube distillate fractionated from the hydrocracked blend was dewaxed to give an oil having the following properties:

|                     |         |
|---------------------|---------|
| Viscosity at 100°F. | 150 SUS |
| Viscosity Index     | 100     |
| Pour Point          | +5°F.   |
| Color (T.R.)        | 9 1/4   |

This distillate was percolated through a bed of silica gel, a bed of alumina, a bed of Filtrol clay, and a bed of a cracking catalyst containing 95 wt.%  $\text{SiO}_2\text{-Al}_2\text{O}_3$  in the proportion of 13%  $\text{Al}_2\text{O}_3$  and 87%  $\text{SiO}_2$ , and 5 wt. percent of a 13-Y zeolite, with heptane as a solvent. The treated oils were then exposed to daylight in clear glass 4 ounce bottles in the presence of air at room temperature. The following data were obtained.

TABLE I

#### Stabilization of Hydrocracked Lubes By Percolation

Conditions 150 Neutral Oil (1 Part W.) Diluted with Heptane (1 Part W.) and Percolated through Absorbent (1 Part W.). Column Washed with Heptane (4 Parts W.).

| Absorbent         | Yield of Oil (Wt. %) | Oil Color (Saybolt) | Days in window until sludge formation |
|-------------------|----------------------|---------------------|---------------------------------------|
| Untreated Oil     | —                    | 9 1/4 T.R.          | 2                                     |
| Cracking Catalyst | 97                   | +35                 | >100                                  |
| Silica Gel        | 95                   | +30                 | 11                                    |
| Alumina (Neutral) | 98                   | +30                 | 12                                    |
| Filtrol Clay      | 98                   | +16                 | 8                                     |

The above data show that percolation through silica gel, alumina or Filtrol clay improved the color of the oil significantly but the daylight stability was increased to only 8 to 12 days, while percolating through the cracking catalyst caused the daylight stability to increase to more than 100 days. A conventional solvent-extracted 150 N lube from a similar crude source has a daylight stability of 21 days.

#### EXAMPLE 2

The experiment of Example 1 was repeated using the same 150 N oil but varying the adsorbent to feed ratio. The following data were obtained.

TABLE 2

#### Stabilization of Hydrocracked Lubes by Percolation

Conditions 150 Neutral Oil (1 Part W.) Diluted with Heptane (1 Part W.) and Percolated Through Cracking Catalyst. Adsorbent then Washed with Heptane.

| Absorbent to Feed Oil Ratio (by weight) | Yield of Treated Oil (Wt. %) | Days in window until sludge formation |
|-----------------------------------------|------------------------------|---------------------------------------|
| 1                                       | 97                           | >100                                  |
| 0.30                                    | 98                           | >41                                   |
| 0.25                                    | 98                           | 10                                    |
| 0.20                                    | 99                           | 9                                     |
| 0.12                                    | 94                           | 7                                     |
| 0.10                                    | 95                           | 8                                     |

The above data show that the daylight stability decreases with decrease in adsorbent to feed oil ratio. A feed oil ratio of less than 0.3 is not suitable if a highly stabilized oil is desired.

| Adsorbent to feed oil ratio (by weight) | Yield of treated oil (wt %) | Days in window until sludge formation |
|-----------------------------------------|-----------------------------|---------------------------------------|
| 0.30                                    | 98                          | >41                                   |

#### EXAMPLE 3

The experiment of Example 1 was repeated and the adsorbent was regenerated by washing with benzene. The regenerated adsorbent was used to treat additional samples of feed. The following data were obtained.

TABLE 3

#### Stabilization of Hydrocracked Lubes by Percolation

#### Regeneration of Adsorbent by Interpercolation Washing

Conditions 150 Neutral Oil (1 Part W.) Diluted with Heptane (1 Part W.) and Percolated through 3B-2 Cracking Catalyst (1 Part W.). Column then Washed with Heptane (4 Parts W.) and Regenerated with Benzene Wash (5 Parts W.). Cycle then repeated.

| Cycle | Yield of Treated Oil (Wt. %) | Days in Window until Sludge Formation |
|-------|------------------------------|---------------------------------------|
| Feed  | —                            | 2                                     |
| 1     | 97                           | >54                                   |
| 2     | 89                           | N/A                                   |
| 3     | 96                           | 53                                    |
| 4     | 96                           | 40                                    |
| 8     | 96                           | >41                                   |

The above data show that the adsorbent column can be repeatedly regenerated by benzene washing and that the hydrocracked oil treated by the regenerated adsorbent was more stable than the conventional reference oil even after the adsorbent column used to treat the hydrocracked oil had been regenerated several times.

#### EXAMPLE 4

The experiment of Example 1 was repeated using a series of higher viscosity hydrocracked oils as feed. The following data were obtained.

TABLE 4

#### Stabilization of Hydrocracked Lubes by Percolation

#### CONDITIONS: AS IN TABLE 2.

| Hydrocracked Feed Oil           | Initial feed color | Yield of treated oil | Color of treated oil (say) | Days in window until sludge formation |
|---------------------------------|--------------------|----------------------|----------------------------|---------------------------------------|
| 150 Neutral Distillate (SAE 10) | 9 1/4              | 97                   | +35                        | >100                                  |
| 600 Neutral Distillate (SAE 30) | 1                  | 94                   | +30                        | >41                                   |
| Bright Stock Residuum           | <1                 | 95                   | 30+                        | >53                                   |

The above data show percolation of higher viscosity grade hydrocracked lubes from the same crude also gave stable oils of much improved color.

## EXAMPLE 5

The hydrocracked oil of Example 1 was slurried with the cracking catalyst adsorbent, with charcoal and with Filtral and the stability of the treated oil determined. The following data were obtained.

TABLE 5 Stabilization of Hydrocracked Lubes by Slurry Contact

| Conditions 150 Neutral Oil Agitated with Adsorbent (10 Wt.%) then Filtered. |                 |                             |                                       |
|-----------------------------------------------------------------------------|-----------------|-----------------------------|---------------------------------------|
| Adsorbent                                                                   | Treat Temp. °F. | Color of Treated oil (T.R.) | Days in window until Sludge Formation |
| Feed Oil                                                                    | —               | 9 1/4                       | 2                                     |
| Cracking Catalyst                                                           | 80              | 14                          | 8                                     |
| Cracking Catalyst (5 Treats of 2 Wt. % Each)                                | 80              | 19 1/4                      | 12                                    |
| Cracking Catalyst                                                           | 150             | 16                          | 8                                     |
| Cracking Catalyst                                                           | 400             | 17                          | 2                                     |
| Charcoal                                                                    | 80              | 8 1/4                       | 2                                     |
| Filtral                                                                     | 400             | 23 1/4                      | 4                                     |
| Filtral (2 Wt.%)                                                            | 80              | 17                          | 4                                     |

The above data show that slurring the oil with the adsorbent followed by filtering improves the stability of the oil somewhat but not to any outstanding degree. The data also show that the cracking catalyst is no better than Filtral when using the slurring technique.

The nature and advantages of the present invention having thus been fully set forth and specific examples of the same given, what is claimed as new, useful and unobvious and desired to be secured by Letters Patent is:

1. A process for forming a lubricating oil fraction resistant to deterioration upon exposure to light and air which comprises contacting a hydrocarbon fraction, at hydrocracking conditions, with a hydrocracking catalyst to form a plurality of fractions including lubricating oil fractions, dewaxing said lubricating oil fractions, percolating said dewaxed lubricating oil fractions with a Y-zeolite, said Y-zeolite being physically combined with an amorphous cracking catalyst containing a major amount of silica and a minor amount of alumina, and recovering a light and air stable lubricating oil fraction.

2. The process of claim 1 in which the hydrocracking step takes place at a temperature between 700° and 900° F., at a pressure above 1,500 psig and a space velocity below 1 V/V/Hr.

3. The process of claim 1 in which said Y-zeolite is faujasite having a silica/alumina mole ratio greater than 3/1 and uniform pore openings of about 6 to 15 Å.

4. The process of claim 2 in which said hydrocracking catalyst is an oxide or sulfide of a metal chosen from the group consisting of Group VB, VIB and VIII of the Periodic System

and mixtures thereof.

5. A process of forming a lubricating oil fraction resistant to deterioration upon exposure to light and air which comprises contacting a hydrocarbon fraction, at hydrocracking conditions, with a hydrocracking catalyst to form a plurality of fractions including lubricating oil fractions, percolating said lubricating oil fractions at temperature below 150° F. with a catalyst comprising silica-alumina gel matrix containing Y-zeolite and recovering a light and air stable lubricating oil fraction.

6. The process of claim 5 in which said silica-alumina gel matrix containing Y-zeolite is a physically combined mixture of an amorphous cracking catalyst containing a major amount of silica and a minor amount of alumina and said Y-zeolite.

15 7. The process of claim 5 in which said Y-zeolite is faujasite having a silica-alumina mole ratio greater than about 3/1 and uniform pore openings of about 6 to 15 Å.

8. The process of claim 5 in which said silica-alumina gel matrix containing Y-zeolite consists of 95 wt. percent of a mixture of  $Al_2O_3/SiO_2$ , in the proportion of 13 wt. %  $Al_2O_3$  and 87 wt. %  $SiO_2$ , with 5 wt. percent faujasite.

9. The process of claim 5 wherein said silica-alumina gel matrix containing Y-zeolite is regenerated by washing with benzene.

25 10. The process of claim 5 wherein said lubricating oil fractions are dewaxed prior to contact with said silica-alumina gel matrix containing Y-zeolite.

11. A process for forming a stabilized lubricating oil fraction resistant to deterioration upon exposure to light and air

30 comprising subjecting a high boiling hydrocarbon fraction to hydrocracking conditions in the presence of a hydrocracking catalyst to form a plurality of fractions including lubricating oil fractions boiling above about 650° F., dewaxing said lubricating oil fractions, percolating at least a portion of said

35 dewaxed lubricating oil fractions through a catalyst comprising silica-alumina gel matrix containing Y-zeolite and recovering a light and air stable lubricating oil fraction.

12. The process of claim 11 in which said silica-alumina gel matrix containing Y-zeolite is a physically combined mixture

40 of an amorphous cracking catalyst containing a major amount of silica and a minor amount of alumina and said Y-zeolite.

13. The process of claim 11 in which said Y-zeolite is faujasite having a silica-alumina mole ratio greater than about 3/1 and uniform pore openings of about 6 to 15 Å.

45 14. The process of claim 11 in which said silica-alumina gel matrix containing Y-zeolite consists of 95 wt. percent of a mixture of  $Al_2O_3/SiO_2$ , in the proportion of 13 wt. %  $Al_2O_3$  and 87 wt. %  $SiO_2$  with 5 wt. percent faujasite.

15. The process of claim 11 wherein said silica-alumina gel matrix containing Y-zeolite is regenerated by washing with benzene.

50 16. The process of claim 11 wherein said percolation is conducted at a temperature less than about 150° F.

\* \* \* \* \*